

Feb. 23, 1937.

H. A. PIGGOTT ET AL

2,071,898

SENSITIZED PHOTOGRAPHIC SILVER HALIDE EMULSIONS

Original Filed May 28, 1931

Fig. 1.

SENSITIVITY RANGE OF PHOTOGRAPHIC  
EMULSION TREATED WITH DYESTUFF OF  
EXAMPLE 1.



Fig. 2.

SENSITIVITY RANGE OF PHOTOGRAPHIC  
EMULSION TREATED WITH DYESTUFF OF  
EXAMPLE 2.



Fig. 3.

SENSITIVITY RANGE OF PHOTOGRAPHIC  
EMULSION TREATED WITH DYESTUFF OF  
EXAMPLE 4.



INVENTORS

Henry Alfred Piggott  
Ernest Harry Rodd

BY

*Arthur T. Davenport*

ATTORNEY

## UNITED STATES PATENT OFFICE

2,071,898

SENSITIZED PHOTOGRAPHIC SILVER  
HALIDE EMULSIONS

Henry Alfred Piggott, Cheadle Hulme, and Ernest Harry Rodd, Brooklands, England, assignors to Imperial Chemical Industries Limited, a corporation of Great Britain

Application May 28, 1931, Serial No. 540,810  
Renewed June 26, 1936. In Great Britain May 31, 1930

9 Claims. (CL 95—7)

This invention relates to photographic sensitizing compositions and to photographic preparations, such as emulsions or plates or films coated with emulsions, comprising such compositions.

It is known that a standard photographic emulsion is sensitive to light rays only within the wavelength range of about 360 to 500 millimicrons, and that by suitable treatment, e. g. by bathing a photographic plate in a dilute solution of a sensitizer, the emulsion becomes sensitive to light of other wave lengths, but it is still a matter of difficulty to increase or decrease the sensitivity at will in any desired degree.

It is an object of the present invention to provide sensitizing compositions which will render photographic emulsions sensitive to light rays in the red and infra-red region of the spectrum. It is a further object of this invention to provide photographic emulsions sensitive to red and infra-red light rays. It is also an object of this invention to provide plates and films coated with such sensitized emulsions.

These objects are achieved according to this invention by the employment of unsymmetrical polymethylene dyestuffs such as can be obtained by condensing a heterocyclic nitrogen compound containing an external reactive methylene group with an intermediate compound obtainable by the process described in our English Patent No. 344,409.

The accompanying drawing illustrates the sensitivity curves of photographic emulsions treated with certain of the unsymmetrical dyestuffs hereinafter described.

Examples of such unsymmetrical dyestuffs are, for instance, the following:

(1) Dyestuff of the formula:



This dyestuff can be obtained by condensing together in acetic anhydride solution 7 parts by weight of 1:3:3-trimethyl-2-methylene-indoline and 16 parts by weight of the product obtained according to Example 2 of English Patent No. 344,409, from quinaldine ethiodide and di-

phenylformamidine. The amount of acetic anhydride used should be 20 parts by weight, and the solution should be boiled under reflux for ten minutes, cooled somewhat, diluted with 50 parts by weight of hot water, and vigorously stirred. The dyestuff separates out and is filtered off and washed.

(2) Dyestuff of the formula:



This dyestuff may be prepared by boiling under reflux a solution in 160 parts by weight of acetic anhydride, to which 5 parts by weight of sodium acetate have been added, of 18 parts by weight of 2:3:3-trimethylindolenine methiodide and 24 parts by weight of the product obtained by condensing 2-methylbenzothiazole ethiodide with diphenylformamidine (cf. Example 5 of English Patent No. 344,409). After boiling for fifteen minutes the mixture is diluted with 150 parts by weight of hot water, and the precipitated dyestuff is purified by lixiviation with ether.

(3) Dyestuff of the formula



This dyestuff may be obtained in a manner exactly similar to (2) but using the product from 2-methylbenzoxazole ethiodide and diphenylformamidine.

(4) Dyestuff of the formula



This dyestuff is analogously obtainable from 2-methylbenzoxazole ethiodide and the product from 2-methylbenzothiazole ethiodide and diphenylformamidine, that is, by boiling under re-

flux in 160 parts of acetic anhydride, to which 5 parts by weight of sodium acetate have been added, 17.92 parts by weight of 2-methylbenzoxazole ethiodide and 26.92 parts by weight of the product from 2-methylbenzylthiazole ethiodide and diphenylformamidine. After boiling for 15 minutes the mixture is diluted with 150 parts by weight of hot water, and the precipitated dyestuff is purified by lixiviation with ether.

Other unsymmetrical dyestuffs of the polymethine series, all obtainable in a similar manner, but containing various heterocyclic nitrogen residues, may also be used according to our invention. Such dyestuffs may be represented by the general formula



where A is a monovalent heterocyclic nitrogen residue of the type



25

in which Ar is an *o*-arylene group, R is alkyl, Y is an acid residue (such as halogen, sulphate, oxalate, etc.) and X stands for the bivalent atom or group  $-O-$ ,  $-S-$ , or  $-CR'2-$  (R' being alkyl),

and B is a divalent heterocyclic nitrogen residue of the type

35



in which Ar, and R have the same significance as before (though not necessarily representing identical groups), whilst Z stands for  $-O-$ ,  $-S-$ , or  $-CR'2-$  (R' being alkyl) and is different from X.

The unsymmetrical polymethine dyestuffs employed in photographic emulsions in accordance with our invention may be described generically by the following formula:

50



in which X represents a member of the oxygen group of elements or dialkyl methylene, Z represents a member of the oxygen group of elements, dialkyl methylene or vinylene and is different from X, Ar and Ar' represent aryl radicals of the benzene series, R and R' represent alkyl radicals, and Y represents the negative radical of an acid.

In carrying our invention into practical effect we treat a photographic emulsion with unsymmetrical polymethine dyestuffs as described above, e. g. by bathing a photographic plate in a dilute aqueous solution of the dyestuff. Preferably a solution of 1 part of dyestuff in 2000 parts of 50% aqueous alcohol is prepared. This stock solution is diluted for use with about 20 parts of water. 100 c. c. of the diluted solution are taken for each full-size photographic plate to be treated, and the plate is immersed in the solution, which is agitated gently, and kept in contact with the plate for a period of about 5 minutes. The plate is then washed with water and dried.

Photographic plates thus treated in accordance with our invention become sensitive as shown in the following table:

| Dyestuff (see formulae above) applied to plate                                                                           | Plate becomes sensitive to wave-length range (in millimicrons) | 5  |
|--------------------------------------------------------------------------------------------------------------------------|----------------------------------------------------------------|----|
| $\begin{array}{c} CH_3 \quad CH_3 \\   \quad   \\ C_6H_5-C-CH=CH-CH=N-C_6H_5 \\   \quad   \\ CH_3 \quad I \end{array}$   | 360-653                                                        | 10 |
| $\begin{array}{c} CH_3 \quad CH_3 \\   \quad   \\ C_6H_5-C-CH=CH-CH=C-O-C_6H_5 \\   \quad   \\ CH_3 \quad I \end{array}$ | 360-600                                                        | 15 |
| $\begin{array}{c} O \\   \\ C_6H_5-C-CH=CH-CH=C-S-C_6H_5 \\   \quad   \\ C_6H_5 \quad I \end{array}$                     | 360-640                                                        | 20 |

It will be understood that these unsymmetrical polymethine dyes may be used in sensitizing any of the usual types of gelatino-silver halide photographic emulsions. These examples are purely illustrative and in no sense intended to limit the scope of the invention.

We claim:

1. Photographic gelatino-silver halide emulsions made sensitive to light of long wave-length by the application of an unsymmetrical polymethine dyestuff having the formula



2. Photographic elements coated with a gelatino-silver halide emulsion made sensitive to light of long wave-length by the application of an unsymmetrical polymethine dyestuff having the formula



3. Gelatino-silver halide photographic emulsions containing an unsymmetrical polymethine dyestuff of the general formula:



wherein X represents a member of the group consisting of the oxygen group of elements and dialkyl methylene; Z represents a member of the group consisting of the oxygen group of elements, dialkyl methylene and vinylene and is different from X, Ar and Ar' represent aryl radicals of the benzene series, R and R' represent alkyl radicals, and Y represents the negative radical of an acid.

4. Gelatino-silver halide photographic emulsions containing an unsymmetrical polymethine dyestuff of the general formula:

5



10 wherein X represents a member of the group consisting of O, S, and dialkyl methylene; Z represents a member of the group consisting of O, S, and dialkyl methylene and is different from X, Ar and Ar' represent aryl radicals of the benzene series, R and R' represent alkyl radicals, and Y represents the negative radical of an acid.

15 5. Photographic elements coated with a gelatino-silver halide emulsion containing an unsymmetrical polymethine dyestuff of the general formula:

25



20 wherein X represents a member of the group consisting of the oxygen group of elements and dialkyl methylene, Z represents a member of the group consisting of the oxygen group of elements, dialkyl methylene and vinylene and is different from X, Ar and Ar' represent aryl radicals of the benzene series, R and R' represent alkyl radicals, and Y represents the negative radical of an acid.

35 6. Photographic elements coated with a gelatino-silver halide emulsion containing an unsymmetrical polymethine dyestuff of the general formula:

40



wherein X represents a member of the group consisting of O, S, and dialkyl methylene, Z represents a member of the group consisting of O, S, and dialkyl methylene and is different from X, Ar and Ar' represent aryl radicals of the benzene series, R and R' represent alkyl radicals, and Y represents the negative radical of an acid.

7. Photographic gelatino-silver halide emulsions containing a dyestuff having the following general formula:

5

10



15

8. Photographic gelatino-silver halide emulsions containing a dyestuff having the following general formula:

20



25

9. Gelatino-silver halide emulsions containing an unsymmetrical polymethine dyestuff of the general formula:

30



35

wherein X and Z represent dissimilar members of the oxygen group of elements, Ar and Ar' represent aryl radicals of the benzene series, R and R' represent alkyl radicals, and Y represents the negative radical of an acid.

HENRY ALFRED PIGGOTT.  
ERNEST HARRY RODD.

40